

# UNITED STATES PATENT OFFICE.

JOHN H. STEVENS, OF NEWARK, NEW JERSEY, ASSIGNOR TO THE CELLULOID MANUFACTURING COMPANY, OF NEW YORK, N. Y.

## MANUFACTURE OF COMPOUNDS OF PYROXYLINE OR NITRO-CELLULOSE.

SPECIFICATION forming part of Letters Patent No. 269,341, dated December 19, 1882.

Application filed June 12, 1882. (No specimens.)

*To all whom it may concern:*

Be it known that I, JOHN H. STEVENS, of the city of Newark, in the county of Essex and State of New Jersey, have invented certain new and useful Improvements in the Manufacture of Compounds of Pyroxyline or Nitro-Cellulose, of which improvements the following is a specification.

In the manufacture of such compounds as those to which my present invention relates it is now well understood that the pyroxyline or nitro-cellulose must be of that class or grade which is designated as "soluble" to distinguish it from other classes or grades which are not soluble, (of which insoluble grades explosive gun-cotton is an example,) as my compounds are intended to be used in the manufacture of various articles formed by molding or shaping the compound in dies, or by cutting, carving, or turning it from a seasoned block or mass.

Heretofore such compounds have been made by dissolving the soluble nitro-cellulose with alcohol and ether, wood-naphtha, and other liquids which are active solvents of such nitro-cellulose at the ordinary temperature; and camphor has been sometimes added to the compound either before or after the solution of the nitro-cellulose by such active liquid solvents. It has also long been known that camphor is of itself an active solvent of nitro-cellulose at the ordinary temperature when the camphor is dissolved in a menstruum—such as alcohol or wood-naphtha—or when a compound is formed of nitro-cellulose, camphor, and certain menstrua which will liquefy the camphor whatever may be the order in which these ingredients are brought together. It is also well known that a mechanical mixture of nitro-cellulose and camphor may be made and afterward subjected to heat and pressure in closed dies, the heat liquefying the camphor and thus developing its solvent action, the camphor being in such cases termed a "latent" solvent; by reason of its inaction until liquefied, whether by heat or by a menstruum. The best practice has been found to demand the mixing of the camphor with the nitro-cellulose and then the addition to that compound of some liquid menstruum which, while not actively develop-

ing the solvent power of the camphor, brings it into a softened condition, which facilitates its liquefaction under heat; and while numerous menstrua have been employed in this way or suggested for this purpose, they have been heretofore, so far as I know, only used practically in conjunction with camphor and for the purpose of liquefying or softening the camphor, as above set forth.

Now, it is the object of my invention to effect the solution, or, as it is more generally designated, the "conversion" of soluble nitro-cellulose by means of latent liquid solvents without necessarily employing camphor in the compound; and by a series of experiments addressed to this end I have ascertained that this may be done in the following manner: The soluble nitro-cellulose should be ground into pulp and dehydrated by hydraulic pressure between absorbent pads, as is well understood. The dried nitro-cellulose is then broken up into small pieces and placed in a vessel which can be tightly closed. To one part, by weight, of this nitro-cellulose I add an equal quantity, by weight, of oil of caraway seed, or oil of hyssop, or oil of sage, or oil of tansy, or oil of cloves, or oil of winter-green, or of mixtures of these oils, each of which I have discovered to be a latent solvent of nitro-cellulose, as hereinafter further explained. The latent liquid solvent being added to the pyroxyline, as above described, the box is tightly closed and the mixture is allowed to stand for, say, about twelve hours; or it may be stirred at intervals to effect a more rapid and thorough absorption of the solvent by the nitro-cellulose, at the end of which period it will be found that the nitro-cellulose has been appreciably softened by the liquid solvent without any active development of the converting process. I then subject the mass to heavy pressure in closed dies at a temperature of about 200° Fahrenheit, and if it is found necessary or desirable to repeat this pressing operation to more thoroughly complete the conversion I again break up the mass into small pieces, and put the compound again in the dies and under heat and pressure, as above described. I have found that the above-specified oils operate in the same manner as

camphor, in that they do not exert their solvent power prematurely, and by their use I am enabled to make a mechanical mixture in the first instances with the advantages of the suspension of the solvent action or converting operation, as is well understood, and then to complete the process by the application of heat and pressure, as above described.

With the nitro-cellulose and latent liquid solvents above specified I compound such coloring-matters or inert substances as may be desired for any special purposes, and the products thus obtained are subjected to the ordinary seasoning operation, after which they may be molded into shapes, in the ordinary manner, under heat and pressure. I subject the compound to heat and pressure in closed dies, as above stated, rather than in open rolls, as is customary in treating such compounds, because I have found that my new latent liquid solvents are better adapted to such treatment; but if I desire to treat the compounds in open rolls or to develop the solvent power of the oils above mentioned at the ordinary temperature, it is only necessary to compound the ingredients as follows: To two parts, by weight, of nitro-cellulose I add two to three parts, by weight, of a mixture of one part, by weight, of either of the oils above mentioned, or of any mixture of those oils compounded together, as hereinbefore described, and two to three parts of alcohol or of wood-naphtha, and this will cause the development of the converting power of the solvent and effect the conversion of the nitro-cellulose even in the cold or more rapidly in the ordinary masticating-rolls, and the product, if the seasoning operation has not been carried too far, will be susceptible of being remolded in the usual way.

Coloring-matters and other inert substances may be incorporated with the mixture of nitro-cellulose and latent liquid solvent, and other

substances may be added to impart any specially desired quality in the product. With the latent liquid solvents above specified it will generally be found necessary to employ coloring-matters, as the compounds made with the above-specified oils are not well adapted for the manufacture of colorless or even of white material.

It will be seen that I have discovered certain latent liquid solvents which may be mechanically mixed with soluble nitro-cellulose, and thus I am enabled to secure the advantages of a latent solvent and a preliminary mechanical mixture without the necessary intervention of any solid converting agent—such as camphor; but it is an additional element of novelty as well as of utility in my improvements, that the use of these latent liquid solvents is entirely compatible with the use of camphor as well as with the use of active solvents—such as wood-naphtha, or ether and alcohol. In other words, my new latent liquid solvents may be added in the hereinbefore-described manner to compounds of pyroxylene and camphor, with an enhancement of the solvent or converting action induced by the development of the latent solvent action of the camphor by the addition of the latent liquid solvent.

Having thus described the nature and objects of my invention, what I claim herein as new, and desire to secure by Letters Patent, is—

As an improvement in the art of manufacturing compounds of pyroxylene or nitro-cellulose, the use of the hereinbefore-specified oils or latent liquid solvents, substantially as set forth.

JOHN H. STEVENS.

Witnesses:

WM. L. BRICE,  
ABRAHAM MANNERS.